

## 1

3,222,195

**STABILIZED ELECTROLESS COPPER SOLUTION**  
 Fred Pearlstein, Philadelphia, Pa., assignor to the United States of America as represented by the Secretary of the Army

No Drawing. Filed Feb. 23, 1962, Ser. No. 175,372

8 Claims. (Cl. 106—1)

(Granted under Title 35, U.S. Code (1952), sec. 266)

The invention described herein may be manufactured and used by or for the Government for governmental purposes without the payment to me of any royalty thereon.

This invention relates to electroless copper solutions and more particularly concerns such solutions having improved resistance to general and rapid decomposition.

Electroless copper solutions, in the main, are Fehling's solutions or variations thereof, having incorporated therein a reducing agent such as formaldehyde. Such solutions generally start decomposing within about 20 minutes after make-up and cannot ordinarily be used for deposition after about 3 hours.

Electroless copper solutions reported in the literature, comprise Fehling's solution and formaldehyde with substantial quantities of complexing agents added thereto, such as sodium carbonate, Versene, and the like. The stability of these solutions, and the rate at which deposits form therefrom leaves much to be desired.

Accordingly, it is an object of this invention to provide a highly stable electroless copper solution.

Another object of the invention is to provide such a solution as aforementioned which requires a very minor amount of an abundantly available compound.

Other and further objects of the invention will be apparent to those skilled in the art upon study of this disclosure.

Briefly, I have found that minor additions of 2-mercaptopbenzothiazole (MBT) to diluted Fehling's solution and formaldehyde produces a marked increase in the stability of the resultant electroless copper solution. More specifically, when 2-mercaptopbenzothiazole is added in amounts ranging between about 0.0005 to 0.008% weight/volume of the original Fehling's solution (the expression "percent weight/volume" being defined as "grams of solute/100 milliliters of solvent" and hence 0.0005 to 0.008% weight/volume equals 5 to 80 milligrams/liter) and to which is added formaldehyde, the resultant solution permits good deposition therefrom at rates faster than any of the known proprietary electroless copper solutions and yet its stability is vastly improved.

In accordance with my invention, Fehling's solution, as specified by the Association of Official Agricultural Chemists, consists of 34.64 g./l.  $\text{CuSO}_4 \cdot 5\text{H}_2\text{O}$ , 173 g./l. rochelle salts.4 $\text{H}_2\text{O}$ , 50 g./l. sodium hydroxide and the balance water. The 2-mercaptopbenzothiazole is readily added to the Fehling's solution from a stock solution consisting of 10 g./l. 2-MBT dissolved in .2 N sodium hydroxide solution. 100 ml. of 36% formaldehyde (containing 12½% methanol as preservative) will then be added to the 2-mercaptopbenzothiazole-Fehling's solution for each liter of original Fehling's solution present. The results of deposition tests conducted at a solution temperature of 25° C. and with varying solutions are shown below in Table I. Each solution was allowed to stand for at least 1 hour before running the tests.

## 2

Table I

[Electroless copper deposition]

| 5  | Electroless copper solution concentration without 2-MBT, percent | 2-MBT, wt./vol., percent | Deposit weight, mg./15 min. on 8 sq. in. | Bath stability | Deposit appearance |
|----|------------------------------------------------------------------|--------------------------|------------------------------------------|----------------|--------------------|
| 10 | 100                                                              | 0.0000                   | 47                                       | Poor           | Poor               |
|    |                                                                  | 0.0005                   | 51                                       | do             | Do                 |
|    |                                                                  | 0.0020                   | 35                                       | do             | Fair               |
|    |                                                                  | 0.0080                   | 39                                       | Fair           | Good               |
|    |                                                                  | 0.0000                   | 36                                       | Poor           | Poor               |
|    | 50                                                               | 0.0005                   | 37                                       | do             | Fair               |
|    |                                                                  | 0.0020                   | 31                                       | Fair           | Good               |
|    |                                                                  | 0.0080                   | 31                                       | Good           | Do                 |
|    |                                                                  | 0.0000                   | 23                                       | Fair           | Do                 |
|    | 25                                                               | 0.0005                   | 21                                       | Good           | Do                 |
|    |                                                                  | 0.0020                   | 18                                       | do             | Do                 |
|    |                                                                  | 0.0080                   | 5                                        | do             | Poor               |

\*The weight per volume percentage of 2-mercaptopbenzothiazole given in Table I above and Table II to follow is based on the undiluted Fehling's solution.

25 Distilled water and reagent grade chemicals were used in preparing the solutions described herein. The electroless copper solution without 2-mercaptopbenzothiazole comprises Fehling's solution and 100 ml. of 36% formaldehyde for each liter of Fehling's solution. At the 50% concentration without 2-mercaptopbenzothiazole, the Fehling's solution is diluted 1 to 1 with distilled water and 100 ml. of 36% formaldehyde added per liter of undiluted Fehling's solution. The 2-mercaptopbenzothiazole may be added directly to the Fehling's solution or the Fehling's solution may be diluted and the 2-mercaptopbenzothiazole added thereto. In any case, the 2-mercaptopbenzothiazole will be added prior to the formaldehyde.

30 Poor bath stability is defined as one in which the bath is substantially decomposed within about 3 hours; a fair bath stability being one which is relatively undecomposed within about 3 hours but almost completely decomposed within 24 hours; and a good bath stability showing little or no decomposition after about 24 hours.

35 A poor deposit appearance is discontinuous or powdery whereas a good deposit appearance is coppery metallic. The appearance of the fair deposit lies therebetween.

40 Deposition tests were performed on a 2-in. x 2-in. cleaned and sensitized Mylar sheet of 0.003 inch thickness.

45 It is apparent from the data presented in Table I that dilution, within the limits shown, improves bath stability but decreases deposition rates. To achieve a good workable compromise between deposition rates and stability, I prefer an electroless copper solution consisting of 40% Fehling's solution with 0.0032% weight/volume of 2-mercaptopbenzothiazole which is based on the undiluted Fehling's solution. To this is added 100 ml. of the aforementioned formaldehyde solution for each liter of the undiluted Fehling's solution present, the resultant solution 50 being used between the range of about 20 to 30° C. In Table II below, comparison data are presented on my stabilized electroless copper solution and three widely used proprietary solutions. The tests were carried out with a bath temperature of about 27° C. using the 40% solution 55 aforescribed.

**3**  
*Table II*

[Deposit weight, mg./15 min. or 8 sq. in.]

| Deposition time      | 2-MBT | Brand X | Brand Y | Brand Z |
|----------------------|-------|---------|---------|---------|
| 15 min.....          | 39    | 16      | 21      | 26      |
| After 180 min.....   | 31    | 12      | 26      | (1)     |
| After 48 hours.....  | 22    | 27      | 22      | .....   |
| After 72 hours.....  | 19    | 24      | .....   | .....   |
| After 192 hours..... | 14    | .....   | .....   | .....   |

<sup>1</sup> Solution completely decomposed.

<sup>2</sup> Poor, discontinuous deposit.

Brand X, Y and Z are modified Fehling's solution-formaldehyde solutions.

It is apparent from the foregoing tables and description that I have provided an electroless copper solution which is more stable than each of the three well-known and widely used commercial solutions. The appearance of my deposit after my solution had been made up for 192 hours was still good and copper was deposited at the rate of about 14 milligrams in 15 minutes. Further, the 2-mercaptopbenzothiazole is incorporated in the Fehling's solution in very minor amounts only and is abundantly available. The principal advantage of my inventive electroless copper solution however resides in its ability to be workable for at least several days thus obviating the necessity for many time consuming solution make-ups.

I claim:

1. In an electroless copper plating solution consisting essentially of Fehling's solution and a reducing agent, the combination therewith of a stabilizing amount of 2-mercaptopbenzothiazole.
2. In an electroless copper plating solution consisting essentially of Fehling's solution and formaldehyde, the combination therewith of a stabilizing amount of 2-mercaptopbenzothiazole.
3. In an electroless copper plating solution consisting

**4**

essentially of Fehling's solution and aqueous formaldehyde solution in the volume ratio of 10 to 1, respectively, the combination therewith of a stabilizing compound consisting of about 5 to 80 milligrams of 2-mercaptopbenzothiazole per liter of undiluted Fehling's solution.

4. An electroless copper plating solution according to claim 3, said solution comprising an additional volume of water ranging from 1 to 3 times the volume of undiluted Fehling's solution.

5. A process for improving stability of an electroless copper plating solution consisting essentially of Fehling's solution and a reducing agent, comprising adding a stabilizing amount of 2-mercaptopbenzothiazole to said electroless copper solution.

6. A process according to claim 5 wherein said reducing agent consists of formaldehyde.

7. A process for improving stability of an electroless copper plating solution consisting essentially of Fehling's solution and aqueous formaldehyde solution in the volume ratio of 10 to 1, respectively, comprising adding to said electroless copper solution 5 to 80 milligrams of 2-mercaptopbenzothiazole per liter of undiluted Fehling's solution.

8. A process according to claim 7 including the step of adding to said electroless copper solution an additional volume of water ranging from 1 to 3 times the volume of undiluted Fehling's solution.

**References Cited by the Examiner**

| UNITED STATES PATENTS |         |          |        |
|-----------------------|---------|----------|--------|
| 2,429,970             | 10/1947 | Wernlund | 204—46 |
| 2,663,684             | 12/1953 | Pierce   | 204—52 |
| 3,033,703             | 5/1962  | Schnble  | 106—1  |

35 ALEXANDER H. BRODMERKEL, *Primary Examiner.*  
JOHN R. SPECK, *Examiner.*